

## UNITED STATES PATENT OFFICE

2,223,473

## SUPERIOR LUBRICATING COMPOSITION

Peter J. Wiezevich, Staten Island, N. Y., now by  
judicial change of name to Peter J. Gaylor, as-  
signor to Standard Oil Development Company,  
a corporation of Delaware

No Drawing. Application October 16, 1937,  
Serial No. 169,459

3 Claims. (Cl. 252—32)

This invention relates to the use of oticica oil and its derivatives for improving the properties of petroleum lubricants and other properties.

Oticica oil is a vegetable drying oil obtained by crushing the seed of a large tree, *Licana rigida* (or the natural order Rosaceae), having northern Brazil as its natural habitat. The seed contains about 60% of the oil which is chemically different from any natural fatty oil so far discovered. This oil contains about 78% of a glyceride of a keto unsaturated acid known as licanic acid and believed to have the formula:



An object of this invention is to employ oticica oil and its derivatives for improving petroleum oils, and especially, lubricating oils. Other objects will become apparent as the description proceeds.

Being highly unsaturated in nature, oticica oil itself has only limited uses in the petroleum field. In small amounts, say 0.1 to 5%, it serves as a powerful oiliness agent and sludge solvent for petroleum lubricants, especially when inhibited against oxidation. It is also useful as a modifying agent in greases and textile lubricants in proportions up to about 5-10%.

This oil is preferably modified in order to widen the scope of its uses. For instance, it may be hydrogenated or partially hydrogenated. A very satisfactory product is obtained when the oil is hydrogenated to a point when only about one double bond per molecule remains. Such a product, as well as the completely hydrogenated material, are highly useful as addition agents in lubricants and fuels in concentrations of 0.1 to 5% or even up to 50% or more. In fact, lubricants can be prepared from the hydrogenated (or partially hydrogenated) oil alone, although it has been found that a cheaper product can be prepared containing about 5-25% mineral oil. Esters of mono or dihydric alcohols such as methyl, ethyl, the butyl and amyl esters and glycols may be used in place of the glyceride which occurs in nature.

When added to petroleum lubricating oils (as in motor or turbine lubricants), this hydro-oticica oil (which term will be employed to designate the partially or completely hydrogenated product) possesses the unusual power to dissolve sludge and to prevent or retard the settling thereof. It also possesses exceptional oiliness and other desirable properties, making it highly suitable as an ingredient in aviation oils, greases,

industrial lubricants, textile oils, as an addition agent to waxes and fuels, etc.

Oticica or hydro-oticica oil may be treated with sulfur, sulfur chlorides, sulfur dioxide, or fluorsulfonic acid to produce sulfurized products having exceptional extreme pressure (E. P.) lubricating action, suitable for hypoid gear lubrication in conjunction with mineral oils or soaps, such as lead or other soaps, etc.

A highly satisfactory agent for improving aviation oils may also be prepared by voltolization of oticica or hydro-oticica oil alone or with mineral lubricating oils and/or other fatty oils such as rapeseed, menhaden, etc. Voltolization is generally accomplished by subjecting the material to the action of a silent electric discharge at room or elevated temperature in a vacuum of about 0.5 atmosphere, using 5000-15,000 volts and 60-1200 cycles. About 5-30% of the voltolized product may be added to the usual mineral oil aviation motor oils, although the voltolized product itself is highly satisfactory for purposes wherein a viscous oil is required.

Thickening of oticica oil or the partially hydrogenated oil may also be accomplished by heat, alone or in presence of sulfur, air, or catalysts such as  $\text{BF}_3$ . In the latter case, heating may be dispensed with and even cooling may be resorted to, due to the violence of the reaction. When heating is employed as the thickening means, it is desirable to carry this treatment out in presence of a vacuum. These products, although not as suitable as the voltolized materials, are satisfactory blending agents for lubricating compositions.

Chlorination of the oil or hydro-oil (with or without materials such as  $\text{SO}_2$ ) gives a viscous product which may be condensed with aromatic compounds, sodium polysulfide, and similar materials to produce pour inhibiting and plastic compounds.

By reacting licanic compounds with hypochlorous acid, chlorhydrins may be produced, from which glycols may be prepared by hydrolysis. Hydroxy licanic acid may be heated to give lactones and lactides. By reaction with maleic anhydride, a condensation product may be prepared suitable for the preparation of resins, etc. Addition of HCl to licanic compounds yields chloro compounds which have especially valuable extreme pressure properties.

When oticica or hydro-oticica oil is hydrolyzed to the licanic acid, glycerol, and other compounds, it is possible to extract the licanic acid (or its salts) by selective solvents such as high

- molecular weight ketones, alcohols, etc. This acid (licanic) may then be converted over into metal soaps, e. g. those of sodium, calcium, aluminum, lead, other heavy metals, and the like, to give products having high solubility in oils and therefore, suitable as addition agents to greases, extreme pressure lubricants, as pigments in paints, in motor oils, insulating oils, textile oils, waxes, rubber and rubber-like products, gasoline, Diesel fuel, etc. These soaps may be used generally in 0.1-5% concentration, although amounts of 10% or more can be employed in special cases where viscous products are required.
- The licanic or hydro-licanic acid can also be esterified with a monohydroxy or polyhydroxy alcohol to give esters suitable as addition agents, to lubricants and fuels. The acid can also be converted to a nitrile or sulfocyanide and employed as an oiliness agent or insecticide in oil solution.
- Oiticica or hydro-oiticica esters or soaps may be hydrogenated strongly to give hydroxy acids, keto alcohols, or glycols. The hydroxy acid may be converted to soap or polymerized to the polyester and added to lubricants, while the keto alcohol or glycol may be employed as solvents or plasticizers or as sludge-solvent agents in lubricants and fuels.

The term "licanic compound" is employed

herein to designate licanic acid, hydro-licanic acid, or compounds or derivatives thereof.

The materials and compositions disclosed herein may be employed in conjunction with other blending agents such as pour inhibitors, polymer 5 thickeners, antioxidants, dyes, paraffin waxes, coating compositions, suspended materials such as graphite, zinc oxide, etc., soaps, extreme pressure agents, corrosion inhibitors, asphalts, resins, rubbers, organo-metallic compounds, fibrous materials, and the like.

This invention is not limited by any theory or specific illustration, but only by the following claims in which it is intended to cover the invention as broadly as the prior art permits. 15

I claim:

1. A composition of matter comprising a petroleum lubricating oil and 0.5-30% of a licanic metal soap soluble in said lubricating oil.
2. A composition of matter according to claim 20 1 in which the metal soap is a soap of a metal of the class of sodium, calcium, aluminum and lead.
3. A composition of matter comprising a petroleum lubricating oil and 0.5-30% of a metal soap 25 of hydrogenated licanic acid, said soap being soluble in said lubricating oil.

PETER J. WIEZEVICH.